

May 6, 1941.

R. L. KREUZ

2,240,789

SHEET PACKING AND GASKET

Filed Feb. 23, 1939

FIG. 1



FIG. 2



FIG. 3



INVENTOR

BY Robert L. Kreuz

J. J. Sticker

ATTORNEY

## UNITED STATES PATENT OFFICE

2,240,789

## SHEET PACKING AND GASKET

Robert L. Kreuz, Detroit, Mich., assignor to Wolverine Fabricating & Manufacturing Company, Inc., a corporation of Michigan

Application February 23, 1939, Serial No. 257,935.

4 Claims. (Cl. 288—34)

My invention pertains to an improved sheet packing material and to improved gaskets made therefrom.

It is an object of my invention to provide an improved sheet packing material which is resistant to the deteriorating effects of oil and other disintegrating fluids and conditions to which such materials are usually exposed, and which has improved characteristics of strength, flexibility and durability and from which improved packing material improved gaskets may be conveniently and cheaply stamped or cut.

It is also an object of my invention to provide an improved sheet packing material comprising a base sheet of chemically vulcanized fiber sheet and the base sheet having on both opposite sides a seating or sealing coat of a material, mixture or compound having a "Thiokol" base or similar commonly known synthetic rubber material, to greatly enhance the seating properties of the surface of the base sheet and effect a good sealing engagement when used as a seal between two adjacent surfaces.

It is a further object of my invention to provide improved gaskets comprising a flexible base sheet having a sealing or seating coating of a "Thiokol" base or a similar synthetic rubber material, the bare edges of the base sheet being exposed at the edges of the gasket, and the base sheet being of a strong, durable, oil-proof, chemically-vulcanized fiber sheet whereby the gasket is not deteriorated by the seepage of oil or other fluids therethrough from the edges.

Further objects and advantages are within the scope of my invention such as relate to the improved characteristics of my product and to economies of manufacture and numerous other features, as will be apparent from a consideration of the specification in conjunction with the drawing illustrating the fabrication of my product, in which:

Fig. 1 is a cross sectional view through a sheet of my improved sheet packing material, the thickness thereof being substantially exaggerated for clearness;

Fig. 2 is a plan view showing a gasket cut or stamped from the sheet packing material; and

Fig. 3 is a sectional view on line 3—3 thereof.

Referring more particularly to Fig. 1 of the drawing, my improved sheet packing material comprises a base sheet 1 of a chemically vulcanized fiber sheet, which I have found possesses unusually desirable characteristics for this purpose. Such base sheet material is readily obtain-

able on the open market. Because of the importance of the characteristics of this base sheet, in the present combination, it will be identified more specifically, although the manufacture of this base sheet, *per se*, is not a part of the present invention.

Such vulcanized fiber sheet, which is used for a base sheet, is usually made from pure cotton, much like pure cotton paper, and it is treated with zinc chloride which changes the nature of the cotton so that it can no longer be detected as such. The chemical is then washed out thoroughly. Thin sheets are then built up and pressed together in a laminated arrangement to fabricate the fiber sheet material. This chemically vulcanized fiber sheet material may also be made by another process in which sulphuric acid is the vulcanizing agent. Such chemically vulcanized laminated sheet material is readily available on the market.

I have found the characteristics of such a base sheet of chemically vulcanized fiber sheet to be quite superior to the properties of other sheet materials previously used for making gaskets, or for similar packing purposes, and a base of such fiber sheet may be used which is very much thinner than is possible with the materials previously used. The chemically vulcanized fiber base sheet is inherently oil-proof. Also this sheet material has very superior strength, flexibility and durability for such purposes, and a very thin base sheet may be used although shown thick in the drawing for clearness.

However, although such fiber sheet has such desirable characteristics, the surface thereof is rather hard and unyielding for use for gaskets and for packing purposes. By applying a sealing or seating coat 3 of a suitable material, mixture, or compound, upon the opposite exposed surfaces 40 of the base sheet 1 of chemically vulcanized fiber sheet, I have found it possible to greatly enhance the seating properties of the surface of such a fiber sheet to provide for good seating engagement with adjacent clamping surfaces between 45 which it may be used as a seal. By such an arrangement it is possible to more effectively and successfully utilize the desirable characteristics of a base sheet of the chemically vulcanized fiber sheet for gaskets and similar purposes.

For the sealing or seating coat 3 on the surfaces of the base sheet 1 of chemically vulcanized fiber sheet, I apply coatings of a "Thiokol" base or a similar synthetic rubber material. The term "Thiokol" is a trade name under which one form 55 of suitable coating material may be readily ob-

tained on the market. This coating material may be coated upon the outer surfaces of the base sheet 1 in any suitable manner as by taking a roll of the fiber sheet, reeling the fiber sheet from one roll to another roll and passing it through an intermediately positioned vat of the coating material, after which it is dried in any suitable manner, as will be readily understood. Such coating material is practically oil proof and the coat 3 thus provided on the outer surfaces of the base sheet 1, gives the surface of a sheet of packing material 6 so formed sealing or seating properties to provide a firm sealing engagement with adjacent surfaces when the material is clamped between two metallic members.

Gaskets 7, as shown in Figs. 2 and 3 or of any other form desired, may be very conveniently and cheaply stamped or cut in any well known manner from a large sheet of my improved packing material, as will be understood. When so formed, the gaskets are ready for use without the necessity of additionally coating the raw edges because the base sheet 1 of the chemically vulcanized sheet material is resistant to oil and other deteriorating effects. The base sheet 1 serves as the gasket material which does not require protection, and the coatings 3 on the opposite side surfaces of the base sheet serve to provide a good sealing seat against any abutting solid surface.

This is also an important property of my improved packing material and of the gaskets made from it, because when a gasket is installed and clamped between two metallic members 9, as represented by the dotted lines in Fig. 3, the inner edge of the base sheet 1 is exposed to the fluid or medium which is to be held under pressure, as indicated by the arrows. As the edges of my gaskets do not require a protective coating, the life of the gasket is not limited by the life of such a protective coating nor is it necessary to exercise particular care to avoid breaking or scratching an edge protective covering when handling or installing the gaskets. When a gasket 7 is installed between two metal members 9, as represented in Fig. 3, the seating or sealing coats 3 of the gasket engage the adjacent

clamping surfaces and form a good sealed joint therewith.

It will be seen that I have provided an improved sheet packing material which may be cheaply manufactured, which has good seating characteristics and desirable properties of strength and durability under the conditions of exposure and use to which such materials are usually subjected, and which may be conveniently and cheaply cut or stamped to form gaskets having similar desirable characteristics.

I claim:

1. A packing and gasket sheet material comprising, a base sheet of a chemically vulcanized fiber, said sheet being substantially incompressible and being resistant to deterioration by oil or the like fluids, and a relatively thin coating of a compressible sealing material applied on both faces of said sheet, said sealing material being resistant to deterioration by oil or the like fluids.

2. A packing and gasket sheet material comprising, a base sheet of a chemically vulcanized fiber, said sheet being substantially incompressible and being resistant to deterioration by oil or the like fluids, and a relatively thin coating of synthetic rubber material applied on opposite faces of said sheet, said synthetic rubber material being resistant to deterioration by oil or the like fluids.

3. A gasket comprising, a base sheet of chemically vulcanized fiber, said sheet being substantially incompressible and being resistant to deterioration by oil or the like fluids, and a relatively thin coating of synthetic rubber material applied on the seating faces of said gasket, said synthetic rubber material being resistant to deterioration by oil or the like fluids.

4. A gasket comprising, a body or base formed of a chemically vulcanized fiber sheet which is substantially incompressible and resistant to deterioration by oil or the like fluids, and a relatively thin coating of oil-resistant synthetic rubber material applied to the seating faces only of said body to provide a resilient, compressible sealing layer on said seating faces.

ROBERT L. KREUZ.